# EUROPEAN PATENT SPECIFICATION

(11) **EP 3 216 883 B1**
(45) Date of publication and mention of the grant of the patent: **28.08.2019**
(21) Application number: 16158893.4
(22) Date of filing: 07.03.2016
(51) Int. Cl.: C22C 5/04, C22F 1/14, A44C 27/00

(54) **IRIDIUM-PLATINUM ALLOY, MACHINED ARTICLE MADE THEREOF AND PROCESSES FOR THEIR PRODUCTION**
IRIDIUM-PLATINLEGIERUNG, DARAUS HERGESTELLTER, MASCHINELL BEARBEITETER GEGENSTAND UND VERFAHREN ZU DEREN HERSTELLUNG
ALLIAGE IRIDIUM-PLATINE, ARTICLE USINÉ CONSTITUÉ DE CELUI-CI ET PROCÉDÉS DE LEUR PRODUCTION

(43) Date of publication of application: 13.09.2017
(73) Proprietor: Heraeus Deutschland GmbH & Co. KG, 63450 Hanau (DE)
(72) Inventor: Schlott, Martin, 63075 Offenbach (DE); Maier, Dirk, 63067 Offenbach (DE); Wald, Verena, 36093 Künzell (DE); Staudt, Nicole, 61169 Friedberg (DE); Lukas, Annette, 63517 Rodenbach (DE)
(74) Representative: Maiwald Patent- und Rechtsanwaltsgesellschaft mbH

(56) References cited:
- CN-A- 101 483 319
- DE-A1-102005 038 772
- YAMABE-MITARAI Y ET AL: "An investigation of phase separation in the Ir-Pt binary system", JOURNAL OF ALLOYS AND COMPOUNDS, ELSEVIER SEQUOIA, LAUSANNE, CH, vol. 484, no. 1-2, 18 September 2009 (2009-09-18), pages 327-334, XP026586446, ISSN: 0925-8388, DOI: 10.1016/J.JALLCOM.2009.04.105 [retrieved on 2009-05-03]
- YOKO YAMABE-MITARAI ET AL: "Solid Solution Hardening Effect of Ir", MATERIALS SCIENCE FORUM, vol. 475-479, 15 January 2005 (2005-01-15) , pages 703-706, XP055294602, ISSN: 0250-9776, DOI: 10.4028/www.scientific.net/MSF.475-479.703

## Description

Iridium is a platinum group metal. Its hardness and melting point are very high. Furthermore, iridium is the second-densest element (after osmium) and one of the most corrosion-resistant metals. Due to these properties, iridium and iridium-containing alloys are interesting materials for a number of applications such as spinnerets, spark plugs, oscillating weights, and jewelry.

WO 2011/034566 describes an item of jewelry made of a metal containing at least 75 wt% iridium.

US 2005/0129960 A1 describes an alloy composition comprising 1-10 at% of Zr and/or Hf, the balance being iridium; and articles which are coated by said alloy composition.

EP 2 281 905 A1 describes an iridium-based metal composition which is free of Zr and Hf and comprises 0.5-30 wt-ppm boron and 0.5 to 20 wt-ppm calcium.

CN 101483319 A describes an iridium-platinum alloy and its use as a spark plug electrode material.

US 2006/0270924 A1 describes an electrode for medical applications, comprising a base body which is coated by a porous Pt-Ir alloy.

DE 10 2005 038 772 A1 describes a wire of oxide dispersion hardened alloy based on platinum and/or palladium. The wire cross-section has an edge zone in which the relatively volatile oxide formers are diluted by at least 25%.

CN 101483319 A describes a sparking-plug electrode material which is made of an alloy containing 90-98 wt% iridium and 2-10 wt% platinum.

However, because of its hardness, brittleness and high melting point, iridium is very difficult to machine, form or work.

The melting point can be lowered by adding platinum, thereby obtaining platinum-iridium alloys. However, such alloys are still very brittle and hard materials, in particular if they are iridium-based (Ir content of more than 50 wt%), and are therefore still very difficult to machine.

If shaped articles are prepared by machining (such as milling) from molded bodies made of a very hard and brittle material, the articles typically show surface defects. In particular along edges generated during the machining process, material may break off. However, for many applications, machined articles having such surface defects (e.g. edge defects) are not acceptable.

An object of the present invention is to provide an iridium-containing alloy which has improved workability and is suitable for preparing shaped articles by machining. If the structure of the shaped article contains edges, the number and size of defects along these edges (e.g. due to material that broke off) should be kept as low as possible.

The object is solved by an iridium-platinum alloy, which contains platinum in an amount of from 25 wt% to 45 wt%, the remainder being iridium and unavoidable impurities, and has an average grain width to height ratio of at least 5.

The shape of grains can be indicated by the grain width to height ratio. If the width to height ratio is close to 1, the grains have a relatively "round" shape, whereas a width to height ratio well above 1 indicates an elongated grain shape. In other words, the higher the aspect ratio is, the more elongated are the grains. Typically, if a material has been subjected to a recrystallization treatment, it contains a high amount of equiaxed grains or may even consist of such grains, i.e. grains having a width to height ratio of close to 1.

In the present invention, it has surprisingly been realized that a molded body which is made of an iridium-platinum alloy having elongated grains so that the average grain width to height ratio is at least 5 can be machined to an article with a reduced number of surface defects. In particular the number and size of edge defects can be significantly reduced.

Preferably, the average grain width to height ratio is at least 8, more preferably at least 10. In a preferred embodiment, the average grain width to height ratio is within the range of from 5 to 25, more preferably from 8 to 20, even more preferably from 10 to 16.

As indicated above, the alloy consists of iridium, platinum and unavoidable impurities. By using iridium of high purity (e.g. a purity of at least 99.9%, more preferably at least 99.99%) and platinum of high purity (e.g. a purity of at least 99.9%, more preferably at least 99.99%) as starting materials, the amount of unavoidable impurities in the final Ir-Pt alloy can be kept on a very low level. Preferably, the iridium-platinum alloy contains less than 200 wt-ppm rhodium. More preferably, the iridium-platinum alloy contains less than 200 wt-ppm rhodium, less than 150 wt-ppm copper, less than 100 wt-ppm calcium, less than 50 wt-ppm boron, and less than 100 wt-ppm iron.

Preferably, the iridium-platinum alloy has an average number of pores per µm² of less than 0.04, more preferably less than 0.03.

Preferably, the iridium-platinum alloy has a hardness of 500 HV1 or less, more preferably 480 HV1 or less.

As will be discussed below in further detail, the iridium-platinum alloy of the present invention is preferably prepared by a process wherein an Ir-Pt cast body is subjected to one or more forming steps such as rolling or forging. Accordingly, it is preferred that the iridium-platinum alloy is a formed iridium-platinum alloy, in particular a rolled or forged iridium-platinum alloy. The formed iridium-platinum alloy can be a disc or a plate. However, other shapes are possible as well.

Furthermore, the present invention relates to a process for preparing the iridium-platinum alloy as described above, which comprises
(i) preparing a cast body from an iridium-platinum melt which consists of iridium, platinum and unavoidable impurities,
(ii) pre-heating the cast body to a temperature Tₚ₋ₕ of from 500°C to less than 1350°C, more preferably from 800°C to less than 1300°C, even more preferably from 1000°C to less than 1250°C; and subjecting the pre-heated cast body to one or more forming steps which are carried out at a temperature T_{f} of from 500°C to less than 1350°C, more preferably from 800°C to less than 1300°C, even more preferably from 1000°C to less than 1250°C, such that the formed iridium-platinum alloy has a degree of recrystallization of less than 30%.

Typically, the casting step (i) includes melting iridium and platinum metal in a furnace, e.g. an induction furnace, so as to prepare an iridium-platinum melt and then casting the melt into a mold. The melt consists of iridium and platinum and unavoidable impurities. The iridium-platinum melt contains the platinum in an amount of from 45 wt% to 25 wt%.

Optionally, the mold is cooled, e.g. water-cooled. It can be preferred that the mold is made of a material having a high thermal conductivity, e.g. at least 200 W/(m*K) or at least 300 W/(m*K) at 20°C, such as copper. A preferred mold is e.g. a water-cooled copper mold.

As known to the skilled person, recrystallisation can be accomplished by thermal treatment (static recrystallization) above the recrystallization temperature, optionally in combination with a forming (e.g. rolling) treatment (dynamic recrystallization). The parameters affecting recrystallization temperature are generally known to the skilled person. The degree of recrystallisation depends *inter alia* on the treatment temperature (i.e. above or below the recrystallization temperature) and duration of treatment.

In the process of the present invention, the pre-heating and the subsequent forming (e.g. rolling) steps are carried out under such conditions that the formed (e.g. rolled) iridium-platinum alloy finally obtained has a degree of recrystallisation of less than 30%. As explained further below, the degree of recrystallization indicates the relative area (in %) of a microsection covered by the recrystallized equiaxed grains.

Based on common general knowledge, the skilled person can identify appropriate process conditions of step (ii) which make sure that the formed (e.g. rolled) iridium-platinum alloy finally obtained has a degree of recrystallisation of less than 30%. Just as an example, the forming (e.g. rolling) of the cast body can be carried out at a temperature which is sufficiently low so as to keep recrystallization on a very low level or is even below the recrystallization temperature. In principle, it is also possible that one or more forming steps are at least partly carried out at a forming temperature above the recrystallization temperature, but the duration of these forming steps at a temperature above the recrystallization temperature is kept sufficiently short so as to avoid any substantial recrystallization.

In a preferred embodiment, the degree of recrystallization of the formed iridium-platinum alloy is less than 20%, more preferably less than 10%, even more preferably less than 5%.

Preferably, at least the final forming step is carried out at a forming temperature T_{f} which is below the recrystallization temperature T_{r-c} of the iridium-platinum alloy. More preferably, each forming step is carried out at a forming temperature which is below the recrystallization temperature of the iridium-platinum alloy. Alternatively, it is also possible that one or more forming steps, except for the final forming step, are carried out at a forming temperature above the recrystallization temperature, but the duration of these forming steps is kept sufficiently short so as to avoid any substantial recrystallization. As known to the skilled person, recrystallization temperature is the temperature at which recrystallization comes to completion in a time that can be commercially realized (typically 1 hour).

The heating time at Tₚ₋ₕ can vary over a broad range. The pre-heating of the cast body at Tₚ₋ₕ can be carried out e.g. for 5-120 minutes or 10 to 90 minutes.

Appropriate forming methods are known to the skilled person. Preferably, the forming of step (ii) is a rolling, a forging, or a combination of both.

Preferably, step (ii) comprises two or more forming steps, e.g. 6 to 30 forming steps, more preferably 10 to 26 forming steps.

Preferably, each forming step is carried out at a forming rate of less than 4.0 s⁻¹, more preferably less than 3.0 s⁻¹, and/or a degree of forming of less than 10.0%, more preferably less than 8.0%.

As known to the skilled person, forming rate can be determined by the following formula $ε = \frac{2 ⁢ πn}{60 \sqrt{r ′}} ⋅ \sqrt{\frac{R}{{H}_{0}}} ⋅ ln \left(\frac{1}{1 - r ′}\right)$ wherein
n is the rotation speed of the roll,
H₀ is the sample thickness before the rolling step,
r' = r/100; r: reduction in sample thickness during the rolling step,
R is the roll radius.

The degree of forming corresponds to the reduction in thickness (in %) of a sample as a result of the forming treatment.

The total degree of forming can be e.g. at least 50%, more preferably at least 65%.

If step (ii) comprises two or more forming steps, it can be preferred that the cast body is re-heated after at least one of these forming steps, so as to avoid that the iridium-platinum alloy cools down too much during the forming (e.g. rolling) treatment. Typically, for re-heating in between two forming steps, the iridium-platinum alloy is transferred from the forming (e.g. rolling) device to an oven, re-heated in the oven to a temperature which is, as explained above, preferably below the recrystallization temperature of the iridium-platinum alloy, and then re-transferred to the forming device so as to continue the forming treatment. The re-heating time can vary over a broad range. The re-heating of the cast body can be carried out e.g. for 0.5 minutes to 20 minutes or 1 minute to 10 minutes. Depending on the size of the cast body, re-heating can be carried out after at least 50% of the forming steps, more preferably after each forming step, except for the final forming step.

Furthermore, the present invention relates to a machined article which contains an the iridium-platinum alloy described above and has a density of at least 21.4 g/cm³.

Preferably, the machined article is an oscillation weight or any other part or component of a clockwork. It may also be a jewelry part.

An oscillating weight is used in a clock and is sometimes also referred to as a rotor. Typically, an oscillating weight or a rotor is a semi-circular disc that freely rotates with each movement of the arm of a clock to automatically wind the mainspring. Its own weight returns it to a vertical position.

Preferably, the machined article (in particular the oscillating weight) has a density of at least 21.6 g/cm³, more preferably at least 21.8 g/cm³.

Preferably, at least 70 wt%, more preferably at least 80 wt%, even more preferably at least 90 wt% of the oscillating weight is made of the iridium-platinum alloy. Most preferably, the oscillating weight consists of the iridium-platinum alloy.

Furthermore, the present invention relates to a process for preparing a machined article, which comprises
- preparing the iridium-platinum alloy by the process described above,
- machining the iridium-platinum alloy.

Preferably, the machined article is an oscillating weight. Typically, the machining includes a milling. Additionally or alternatively, the machining may include a drilling, a turning or other commonly known machining steps.

### Measuring methods

The parameters referred to in the present invention are determined as follows:

### Preparation of microsections for microstructure analysis

The microsection was taken perpendicular to the rolled surface and in (i.e. parallel to) the rolling direction. The material was embedded under vacuum into an epoxy resin. The surface to be analysed was ground and polished. For grinding, the wet grinding machine Labo-Pol-25 of Struers was used at 200 rpm in eight grinding steps (120, 320, 500, 800, 1200, 1500, 2400, and 4000). Polishing was carried out with the device LaboPol-5 of Struers (250 rpm) up to a fineness of 1 µm (diamond polishing paste). Subsequently, the samples were electrolytically etched with 20% KCN.

### Average grain width to height ratio

The average ratio of grain width to grain height of the samples was determined as follows:
As already mentioned above, if the sample was rolled, the microsection was taken perpendicular to the rolled sample surface and parallel to the rolling direction. If two or more rolling steps were carried out on the sample surface and the rolling direction varied, the microsection was prepared in rolling direction of the final rolling step. On the microsection, at least two sub-sections were selected, each sub-section containing at least 40 grains. For each grain, its width (i.e. its maximum dimension in rolling direction) and its height (i.e. its maximum dimension perpendicular to the rolling direction) were determined using a light microscope (Olympus PMG3) with a scale bar. For each grain, the ratio of grain width to grain height was determined. Finally, from the ratio values of the individual grains, the average grain width to height ratio was determined as the arithmetic mean value.

### Average degree of recrystallization

A microsection was prepared as described above, i.e. perpendicular to the rolled sample surface and in rolling direction. On the microsection, at least two sub-sections were selected, each sub-section containing at least 40 grains. For each subsection, the relative area (in %) which was covered by recrystallized (i.e. equiaxed) grains was determined. The relative area covered by the recrystallized grains can be determined via image analysis software. As recrystallized grains, those were considered which have a grain width to height ratio of from 0.75 to 1.25. Finally, from the values of the sub-sections, the average degree of recrystallization was determined as the arithmetic mean value.

### Number of pores per µm²

Using a light microscope (magnification 500x), the number of pores over an area of 50x50 µm² were counted and then converted to the number of pores per 1 µm². In total, this was done for 10 different areas on the microsection, and the average number of pores was calculated as the arithmetic mean value.

### Density

Density was determined according to the Archimedes' principle via the buoyancy force. The sample weight was measured with the balance SB23001 DeltaRange of Mettler Toledo. Then, the weight of the sample in water was determined. The amount of water soaked up was determined by weighing the wet sample. For calculating the density of the sample, a density of water at 22.5°C of 0.99791 g/cm³ was assumed. The density was calculated as follows: $Density \left(g/{cm}^{3}\right) = 0.99791 \left(g/{cm}^{3}\right) \times \left({SW}_{dry}/\left({SW}_{wet}-{SW}_{water}\right)\right)$ wherein
SW_{dry} is the weight (in g) of the dry sample,
SW_{wet} is the weight (in g) of the wet sample,
SW_{water} is the weight of the sample in water.

### Hardness

Hardness of the ground samples was determined under a load of HV1 using the device Zwick Roell ZHµ.

### Amount of impurities

The amount of impurities was determined by glow discharge lamp (GDL) using the device GD Profiler HR of Horiba-Jobin-Yvon. Sample excitation was effected by sputtering and an emission spectrum was obtained. By comparing the intensities of the emission lines to calibrated standards, the amounts of the impurities in the ppm-range was determined.

### Examples

In the following examples, iridium-platinum alloys were prepared which differ in their average grain width to height ratios. From these Ir-Pt alloys, oscillating weights were prepared by milling and these machined articles were inspected for defects at their edges.

### Inventive Example 1 (IE1): Ir-Pt alloy, Pt content: 40 wt%

Appropriate amounts of iridium (3N purity) and platinum (3N purity) for obtaining an Ir-Pt alloy having a Pt content of 40 wt% were melted under argon at 2200°C in an induction furnace using a ZrO₂ crucible. The iridium-platinum melt was cast into a water-cooled copper mold. Upon solidification, an iridium-platinum cast body was obtained. The cast body was removed from the mold and casting wrinkles on its surface were removed by milling.

The cast body was pre-heated at 1200°C for 30 minutes in an oven under air atmosphere. Then, the pre-heated cast body was subjected to 19 rolling steps. After each rolling step, with the exception of the final rolling step, the cast body was transferred from the rolling machine to an oven, re-heated at a temperature of 1200°C for about 5 minutes, and then re-transferred to the rolling machine for carrying out the next rolling step.

Thickness of the cast body prior to the rolling treatment and after each rolling step as well as reduction in thickness (in mm and in %) and forming rates of each rolling step are listed below in Table 1.

**Table 1: Forming rates and reduction in thickness**

| Rolling step | Thickness [mm] | Reduction in thickness [mm] | Reduction in thickness [%] | Forming rate [1/s] |
|---|---|---|---|---|
| 0 (i.e. prior to rolling) | 12 | 0 | 0 | |
| 1 | 11,4 | 0,6 | 5 | 1,34 |
| 2 | 10,6 | 0,8 | 7,02 | 1,64 |
| 3 | 9,25 | 0,6 | 5,66 | 1,52 |
| 4 | 8,50 | 0,75 | 7,50 | 1,82 |
| 16 | 3,7 | 0,3 | 7,50 | 2,88 |
| 17 | 3,5 | 0,2 | 5,41 | 2,52 |
| 18 | 3,3 | 0,2 | 5,71 | 2,66 |
| 19 | 3,1 | 0,2 | 6,06 | 2,83 |

As known to the skilled person, forming rate can be determined by the following formula $ε = \frac{2 ⁢ πn}{60 \sqrt{r ′}} ⋅ \sqrt{\frac{R}{{H}_{0}}} ⋅ ln \left(\frac{1}{1 - r ′}\right)$ wherein
n is the rotation speed of the roll,
H₀ is the sample thickness before the rolling step,
r' = r/100; r: reduction in sample thickness during the rolling step,
R is the roll radius.

Rotation speed of the roll was 22 rpm and roll radius was 155 mm.

After the final rolling step, a plate of 220x50x3 mm was obtained. Perpendicular to the rolled sample surface, an etched microsection was prepared. An optical image of said etched microsection is shown in Figure 1.

The Ir/Pt40 alloy had an average grain width to height ratio of 12.5. The number of pores was 0.01 per µm². Pore size values were well below 5 µm. The degree of recrystallization was very low (well below 30%).

Impurities were present in low amounts: Rh < 200 wt-ppm, Cu < 150 wt-ppm, Ca < 100 wt-ppm, B < 50 wt-ppm, Fe < 100 ppm.

The sample had a hardness of 475 HV1 and a density of 22.0 g/cm³.

The cast body made of the Ir/Pt40 alloy was machined to a balance wheel by milling. The edges of the milled article were inspected for defects having a size of > 10 µm. However, no defects were detected.

### Comparative Example 1 (CE1): Ir-Pt alloy, Pt content: 40 wt%

Appropriate amounts of iridium (3N purity) and platinum (3N purity) for obtaining an Ir-Pt alloy having a Pt content of 40 wt% were melted under argon at 2200°C in an induction furnace using a ZrO₂ crucible. The iridium-platinum melt was cast into a water-cooled copper mold. Upon solidification, an iridium-platinum cast body was obtained. The cast body was removed from the mold and casting wrinkles on its surface were removed by milling.

The cast body was heated at 1400°C for 30 minutes in an oven under air atmosphere. Then, the heated cast body was subjected to 19 rolling steps. After each rolling step, with the exception of the final rolling step, the cast body was re-heated at a temperature of 1400°C for about 4 minutes. Apart from the higher temperature, rolling conditions were identical to those of Inventive Example 1. Accordingly, thickness of the cast body prior to the rolling treatment and after each rolling step as well as reduction in thickness (in mm and in %) and forming rates of each rolling step were corresponding to those listed above in Table 1.

After the final rolling step, a plate of 220x50x3 mm was obtained. Perpendicular to the rolled sample surface, an etched microsection was prepared. An optical image of said etched microsection is shown in Figure 2.

The Ir/Pt40 alloy of CE1 was a mixture of grains having a width to height ratio of close to 1 and slightly elongated grains having a width to height ratio of up to 5. Thus, the average grain width to height ratio was well below 5. The number of pores was 0.05 per µm². A significant degree of recrystallization of more than 30% was detected.

Similar to Inventive Example 1, impurities were present in low amounts: Rh < 200 wt-ppm, Cu < 150 wt-ppm, Ca < 100 wt-ppm, B < 50 wt-ppm, Fe < 100 ppm.

The sample of CE1 had a hardness of 485 HV1 and a density of 22.0 g/cm³.

Under the same machining conditions as used in Inventive Example 1, the cast body made of the Ir/Pt40 alloy of CE1 was machined to a balance wheel by milling. The edges of the milled article were inspected for defects having a size of > 10 µm. A significant number of such large size edge-located defects were detected.

The results of Inventive Example 1 and Comparative Example 1 are summarized in Table 2.

**Table 2: Properties of the samples of IE1 and CE1**

| | Inventive Example 1 | Comparative Example 1 |
|---|---|---|
| Average grain width to height ratio | 12.5 | <5 |
| Number of pores/µm²) | 0,01 | 0,05 |
| Hardness (HV1) | 475 | 485 |
| Density (g/cm³) | 22,04 | 22,0 |
| Number of large size (> 10 µm) edge-located defects in a milled article made of the Ir/Pt alloy | 0 | > 10 |

As demonstrated by the Examples, a molded body made of an iridium-platinum alloy having elongated grains can be machined to an article with a reduced number of surface defects. In particular the number and size of edge defects can be significantly reduced.

## Claims

1. An iridium-platinum alloy, which contains platinum in an amount of from 25 wt% to 45 wt% or less, the remainder being iridium and unavoidable impurities, and has an average grain width to height ratio of at least 5.

2. The iridium-platinum alloy according to claim 1, wherein the average grain width to height ratio is within the range of from 5 to 25.

3. The iridium-platinum alloy according to claim 1 or 2, having an average number of pores per µm² of less than 0.04; and/or having a hardness of 500 HV1 or less, more preferably 480 HV1 or less.

4. The iridium-platinum alloy according to one of the preceding claims, containing less than 200 wt-ppm rhodium, less than 150 wt-ppm copper, less than 100 wt-ppm calcium, less than 50 wt-ppm boron, and less than 100 wt-ppm iron.

5. The iridium-platinum alloy according to one of the preceding claims, which is a rolled or forged iridium-platinum alloy, preferably having the shape of a disc or plate.

6. A process for preparing the iridium-platinum alloy according to one of the claims 1 to 5, which comprises
(i) preparing a cast body from an iridium-platinum melt which consists of iridium, platinum and unavoidable impurities,
(ii) pre-heating the cast body to a temperature Tₚ₋ₕ of from 500°C to less than 1350°C, and subjecting the pre-heated cast body to one or more forming steps which are carried out at a temperature T_{f} of from 500°C to less than 1350°C, such that the formed iridium-platinum alloy has a degree of recrystallization of less than 30%.

7. The process according to claim 6, wherein at least the final forming step is carried out at a forming temperature T_{f} which is below the recrystallization temperature; and/or wherein pre-heating of the cast body is carried out at a temperature Tₚ₋ₕ which is below the recrystallization temperature.

8. The process according to claim 6 or 7, wherein the cast body is pre-heated to a temperature Tₚ₋ₕ of from 800°C to less than 1300°C, even more preferably from 1000°C to less than 1250°C; and the one or more forming steps are carried out at a temperature T_{f} of from 800°C to less than 1300°C, even more preferably from 1000°C to less than 1250°C.

9. The process according to one of the claims 6 to 8, wherein the forming of step (ii) is a rolling, or a forging or a combination thereof; and/or step (ii) comprises two or more forming steps, more preferably from 6 to 30 forming steps.

10. The process according to one of the claims 6 to 9, wherein each forming step is carried out at a forming rate of less than 4.0 s⁻¹, more preferably less than 3.0 s⁻¹, and/or a degree of forming of less than 10.0%, more preferably less than 8.0%.

11. A machined article, which contains the iridium-platinum alloy according to one of the claims 1 to 5 and has a density of at least 21.4 g/cm³.

12. The machined article of claim 11, which is an oscillating weight.

13. The machined article according to claim 11 or 12, wherein at least 80 wt%, more preferably at least 90 wt% of the machined article is made of the iridium-platinum alloy.

14. A process for preparing a machined article, which comprises
- preparing an iridium-platinum alloy according to the method of one of the claims 6 to 10,
- subjecting the iridium-platinum alloy to machining, in particular milling.

## Patentansprüche

1. Ididium-Platin-Legierung, die Platin in einer Menge von 25 Gew.-% bis 45 Gew.-% oder weniger enthält, wobei der Rest Iridium und unvermeidbare Verunreinigungen ist, und ein mittleres Verhältnis von Kornbreite zu -höhe von wenigstens 5 aufweist.

2. Iridium-Platin-Legierung gemäß Anspruch 1, wobei das mittlere Verhältnis von Kornbreite zu -höhe in dem Bereich von 5 bis 25 liegt.

3. Iridium-Platin-Legierung gemäß Anspruch 1 oder 2 mit einer mittleren Zahl von Poren pro µm² von weniger als 0,04; und/oder mit einer Härte von 500 HV1 oder weniger, bevorzugter 480 HV1 oder weniger.

4. Iridium-Platin-Legierung gemäß einem der vorstehenden Ansprüche, die weniger als 200 Gew.-ppm Rhodium, weniger als 150 Gew.-ppm Kupfer, weniger als 100 Gew.-ppm Calcium, weniger als 50 Gew.-ppm Bor und weniger als 100 Gew.-ppm Eisen enthält.

5. Iridium-Platin-Legierung gemäß einem der vorstehenden Ansprüche, die eine gewalzte oder geschmiedete Iridium-Platin-Legierung ist, vorzugsweise mit der Form einer Scheibe oder Platte.

6. Verfahren zur Herstellung der Iridium-Platin-Legierung gemäß einem der Ansprüche 1 bis 5, umfassend
(i) Herstellen eines Gusskörpers aus einer Iridium-Platin-Schmelze, die aus Iridium, Platin und unvermeidbaren Verunreinigungen besteht,
(ii) Vorheizen des Gusskörpers auf eine Temperatur Tₚ₋ₕ von 500 °C bis weniger als 1350 °C und Unterwerfen des vorgeheizten Gusskörpers an einen oder mehrere Formgebungsschritte, die bei einer Temperatur T_{f} von 500 °C bis weniger als 1350 °C durchgeführt werden, so dass die gebildete Iridium-Platin-Legierung einen Rekristallisationsgrad von weniger als 30 % aufweist.

7. Verfahren gemäß Anspruch 6, wobei wenigstens der letzte Formgebungsschritt bei einer Formgebungstemperatur T_{f} durchgeführt wird, die unter der Rekristallisationstemperatur liegt; und/oder wobei Vorwärmen des Gusskörpers bei einer Temperatur Tₚ₋ₕ durchgeführt wird, die unter der Rekristallisationstemperatur liegt.

8. Verfahren gemäß Anspruch 6 oder 7, wobei der Gusskörper bei einer Temperatur Tₚ₋ₕ von 800 °C bis weniger als 1300 °C, noch bevorzugter von 1000 °C bis weniger als 1250 °C, vorgewärmt wird; und der eine oder die mehreren Formgebungsschritte bei einer Temperatur T_{f} von 800 °C bis weniger als 1300 °C, noch bevorzugter von 1000 °C bis weniger als 1250 °C, durchgeführt werden.

9. Verfahren gemäß einem der Ansprüche 6 bis 8, wobei die Formgebung von Schritt (ii) Walzen, Schmieden oder eine Kombination davon ist; und/oder Schritt (ii) einen oder mehrere Formgebungsschritte, bevorzugter von 6 bis 30 Formgebungsschritte, umfasst.

10. Verfahren gemäß einem der Ansprüche 6 bis 9, wobei jeder Formgebungsschritt mit einer Formgebungsrate von weniger als 4,0 s⁻¹, bevorzugter weniger als 3,0 s⁻¹, und/oder einem Formgebungsgrad von weniger als 10,0 %, bevorzugter weniger als 8,0 %, durchgeführt wird.

11. Bearbeiteter Gegenstand, der die Iridium-Platin-Legierung gemäß einem der Ansprüche 1 bis 5 enthält und eine Dichte von wenigstens 21,4 g/cm³ aufweist.

12. Bearbeiteter Gegenstand gemäß Anspruch 11, der eine Schwungmasse ist.

13. Bearbeiteter Gegenstand gemäß Anspruch 11 oder 12, wobei wenigstens 80 Gew.-%, bevorzugter wenigstens 90 Gew.-%, des bearbeiteten Gegenstands aus der Iridium-Platin-Legierung bestehen.

14. Verfahren zur Herstellung eines bearbeiteten Gegenstands, umfassend
- Herstellen einer Iridium-Platin-Legierung gemäß dem Verfahren gemäß einem der Ansprüche 6 bis 10,
- Unterwerfen der Iridium-Platin-Legierung an Bearbeitung, insbesondere Fräsen.

## Revendications

1. Alliage d'iridium-platine, qui contient du platine en une quantité de 25 % en poids à 45 % en poids ou moins, le reste étant de l'iridium et des impuretés inévitables, et qui a un rapport moyen de la largeur à la hauteur des grains d'au moins 5.

2. Alliage d'iridium-platine selon la revendication 1, dans lequel le rapport moyen de la largeur à la hauteur des grains est dans la plage de 5 à 25.

3. Alliage d'iridium-platine selon la revendication 1 ou 2, ayant un nombre moyen de pores par µm² inférieur à 0,04 ; et/ou ayant une dureté inférieure ou égale à 500 HV1, plus préférablement inférieure ou égale à 480 HV1.

4. Alliage d'iridium-platine selon l'une des revendications précédentes, contenant moins de 200 ppm en poids de rhodium, moins de 150 ppm en poids de cuivre, moins de 100 ppm en poids de calcium, moins de 50 ppm en poids de bore et moins de 100 ppm en poids de fer.

5. Alliage d'iridium-platine selon l'une des revendications précédentes, qui est un alliage d'iridium-platine laminé ou forgé, de préférence ayant la forme d'un disque ou d'une plaque.

6. Procédé pour la préparation de l'alliage d'iridium-platine selon l'une des revendications 1 à 5, qui comprend
(i) la préparation d'un corps coulé à partir d'une masse fondue d'iridium-platine qui est constituée d'iridium, de platine et d'impuretés inévitables,
(ii) le préchauffage du corps coulé à une température Tₚ₋ₕ de 500 °C à moins de 1350 °C et le fait de soumettre le corps coulé préchauffé à une ou plusieurs étapes de formage qui sont mises en oeuvre à une température T_{f} de 500 °C à moins de 1350 °C, de façon telle que l'alliage d'iridium-platine formé a un degré de recristallisation inférieur à 30 %.

7. Procédé selon la revendication 6, dans lequel au moins l'étape de formage final est mise en oeuvre à une température de formage T_{f} qui est au-dessous de la température de recristallisation ; et/ou dans lequel le préchauffage du corps coulé est mis en oeuvre à une température Tₚ₋ₕ qui est au-dessous de la température de recristallisation.

8. Procédé selon la revendication 6 ou 7, dans lequel le corps coulé est préchauffé à une température Tₚ₋ₕ de 800 °C à moins de 1300 °C, encore plus préférablement de 1000 °C à moins de 1250 °C ; et la ou les étapes de formage sont mises en oeuvre à une température T_{f} de 800 °C à moins de 1300 °C, encore plus préférablement de 1000 °C à moins de 1250 °C.

9. Procédé selon l'une des revendications 6 à 8, dans lequel le formage de l'étape (ii) est un laminage ou un forgeage ou une combinaison de ceux-ci ; et/ou l'étape (ii) comprend deux ou plus de deux étapes de formage, plus préférablement de 6 à 30 étapes de formage.

10. Procédé selon l'une des revendications 6 à 9, dans lequel chaque étape de formage est mise en oeuvre à une vitesse de formage inférieure à 4,0 s⁻¹, plus préférablement inférieure à 3,0 s⁻¹, et/ou un degré de formage inférieur à 10,0 %, plus préférablement inférieur à 8,0 %.

11. Article usiné, qui contient l'alliage d'iridium-platine selon l'une des revendications 1 à 5 et qui a une masse volumique d'au moins 21,4 g/cm³.

12. Article usiné selon la revendication 11, qui est une masse oscillante.

13. Article usiné selon la revendication 11 ou 12, au moins 80 % en poids, plus préférablement au moins 90 % en poids de l'article usiné étant constitué de l'alliage d'iridium-platine.

14. Procédé pour la préparation d'un article usiné, qui comprend
- la préparation d'un alliage d'iridium-platine selon le procédé de l'une des revendications 6 à 10,
- le fait de soumettre l'alliage d'iridium-platine à un usinage, en particulier un fraisage.
